

Patented Jan. 5, 1937

2,066,918

# UNITED STATES PATENT OFFICE

2,066,918

## LIGHT-SENSITIVE MATERIAL AND A PROCESS OF PRODUCING PICTURES

Gottlieb von Poser and Robert Franke, Wiesbaden, Germany, assignors to Kalle & Co. Aktiengesellschaft, Wiesbaden-Biebrich, Germany, a corporation of Germany

No Drawing. Application September 13, 1932, Serial No. 633,016. In Germany September 21, 1931

14 Claims. (Cl. 95—6)

The present invention relates to light-sensitive material, capable of yielding positive pictures from a negative original and to a process of producing pictures therefrom.

5 One object of the present invention is light-sensitive materials which are prepared by applying silver salts in mixture with light-sensitive diazo compounds upon or in a suitable support. The light-sensitive materials thus obtained yield rather good silver-pictures, after exposure to light, after-treatment with alkalies or the like and fixation. All silver salts which are water-soluble may be used for the present invention, as for instance, silver nitrate. As diazo compounds there may be used all such stable, light-sensitive diazo compounds, as yield, when exposed to light, decomposition products capable of exercising a reducing action on the exposed silver salt. Such diazo compounds are, for instance, amino diazo compounds of the benzene or naphthalene series, which may be substituted in the nucleus or in the amino group, for instance, by alkyl, hydroxy groups, carboxy groups, sulfo groups, halogen or the like. The amino diazo compounds of the benzene series useful in the present invention are preferably obtained from amino compounds of the following general formula: R—NH<sub>2</sub> where 10 in R stands for a benzene- or a naphthalene-radical being substituted in the nucleus by hydroxy, halogen, alkyl, oxalkyl, oxaryl, oxaralkyl, an amino group, a substituted amino group, a carboxy group or a sulfonic acid group. The diazo compounds may be used as such, or in the form of salts, such as, for instance, sulfates, chlorobenzene-sulfonates, or the like.

Another object of the present invention is the process of preparing pictures from the light-sensitive materials described above. The material is exposed to light under a design and thereby is obtained a positive picture from a negative design and vice versa. After exposure to light, the picture is treated with alkali or substances having an alkaline action, such as, for instance, ammonia, soda, borax, sodium acetate or the like, 15 alone or in mixture with one another, and then subjected to a washing or fixating process, for instance, with sodium thiosulfate, in order to remove the substances which have not reacted. The formation of the picture probably takes place 20 in such a way, that the light acts upon the diazo compound which is rather sensitive to light, whereby the latter yields a decomposition product. This product, which preferably has a reducing action, acts upon the silver salt with the 25 formation of metallic silver, which action is completed by the subsequent treatment with a substance of alkaline action. The silver picture thus obtained is then fixed in the usual manner. The new process has the rather important advantage 30 that the silver picture is obtained at once after

the exposure to light and that a separate development process, as is necessary in the usual photographic processes, is not required. A further advantage lies in the rapidity of the formation of the picture, caused by the great light-sensitivity of the diazo compounds used. Because of this fact it is possible to use silver salts which are not very sensitive to light. Thus also silver compounds which are of small value for photographic purposes, such as silver nitrate, can be used in the present process.

5 The light-sensitive material can be prepared according to one of the methods usually employed in diazo type printing and in photography. It is 10 possible, for instance, simply to apply an aqueous or an aqueous-alcoholic solution of the mixtures of diazo compounds and silver salts on a base, for instance, paper, gelatinized paper or a film from a cellulose derivative or cellulose hydrate; the preservatives known from the photoprinting industry, such as, for instance, metal salts, acids, dextrose, starch etc. may be added. The light-sensitive substances can also be applied on a base in a colloid, such as, for instance, gelatine, in a 15 manner customary in the photographic industry.

20 The proportion of the diazo salts and silver salts may vary within wide limits. According to the 25 quantities of the two constituents, the kind of the diazo compounds, the silver salts and the substances added to the layer, and according to the after-treatment with alkaline agents, the tones vary from brown to black, and the gradation of the pictures varies, too. Other light-sensitive substances, such as, for instance, ferric ammonium citrate, may be mixed with the layers, 30 whereby more dark brown pictures are obtained. Ferric ammonium citrate has already been used together with silver salts for the preparation of 35 light-sensitive layers, but when using the same quantities of silver, there cannot be obtained such rich and deep tones as according to the 40 present process.

45 The following examples illustrate the invention.

(1) 10 parts of the chlorobenzenesulfonate of the diazotized 1-amino-4-diethylaminobenzene-2-carboxylic acid



50 and 8 parts of silver nitrate are dissolved, while adding 4 parts of tartaric acid, in 250 parts of water. The solution is applied on photographic 55 crude paper. On exposure to light under a nega- 60

tive design, a red picture is obtained which is already well visible. After bathing for a short time in a solution of sodium carbonate of 1% strength, the color of the picture turns to black.

- 5 It is fixed for 1 minute in a solution of 4% strength of thiosulfate and washed with water. By addition of 5 parts of gelatine, pictures of a steeper gradation are obtained. Instead of the 1-diazo-4-diethylaminobenzene-2-carboxylic acid 10 there may also be used with the same effect the corresponding sulfonic acid. Instead of paper, there may, of course, also be used other bases, such as, for instance, a film.

- (2) 10 parts of 4-diazodiphenylaminesulfate 15 obtained by diazotizing aminodiphenylamine of the following formula



20

25

- 30 in a sulfuric acid solution, and 12 parts of silver nitrate are dissolved in 350 parts of water. The papers to which this solution is applied are exposed to light, treated with a solution of 3% strength of borax and fixed with a solution of 4% strength of thiosulfate. When using ordinary 35 paper, yellowish-brown to brown pictures are obtained, and when using baryta paper, strong black pictures are obtained. Instead of 4-diazodiphenylaminesulfate there may be used a corresponding quantity of the diazo compound of 40 1-amino-4-ethylaminonaphthalene.

(3) 10 parts of the chlorobenzenesulfonic acid compound of para-phenylenediamine of the following formula



45

50

- 55 one amino group of which is diazotized in a sulfuric acid solution, are dissolved together with 6 parts of silver nitrate in 400 parts of water. When this solution is applied on paper, the latter 60 yields, on exposure to light and after a treatment with sodium carbonate, pure brown pictures.

- (4) 10 parts of the chlorobenzenesulfonate of the diazo compound of para-aminophenol



- 65 are dissolved together with 10 parts of silver nitrate in 250 parts of water and the solution is applied on paper. After exposure to light a red picture is obtained which assumes a deep brown tone upon being subjected to a short treatment with gaseous ammonia and subsequently washed 70 with water.

- (5) 15 parts of ortho-dimethylaminoaniline



5

are diazotized in a sulfuric acid solution. After neutralization of the acid, the solution is mixed with 12 parts of silver nitrate, and applied on 10 paper. After exposure to light and a short treatment with a solution of 1% strength of sodium carbonate, yellowish-brown pictures are obtained.

We claim:

1. Light-sensitive material sensitized by means of a mixture of a water-soluble silver salt and a light-sensitive aromatic amino diazo compound of the benzene series, the silver salt being used in sufficient quantity to produce a silver picture.

2. Light-sensitive material sensitized by means of a mixture of silver nitrate and 1-diazo-4-diethylaminobenzene-2-carboxylic acid.

3. Light-sensitive material sensitized by means of a mixture of silver nitrate and 4-diazodiphenylamine.

4. Light-sensitive material sensitized by means of a mixture of silver nitrate and 1-diazo-4-aminobenzene.

5. A process of preparing positive pictures from a negative design, which comprises exposing to light under the design a light-sensitive material sensitized by means of a mixture of a water-soluble silver salt and a light-sensitive aromatic amino diazo compound of the benzene series, the silver salt being used in sufficient quantity to produce a silver picture, subjecting the picture thus obtained to the action of a substance of alkaline action and then to a fixing process.

6. A process of preparing positive pictures from a negative design, which comprises exposing to light under the design a light-sensitive material sensitized by means of a mixture of silver nitrate and 1-diazo-4-diethylaminobenzene-2-carboxylic acid, subjecting the picture thus obtained to the action of a substance of alkaline action and then to a fixing process.

7. A process of preparing positive pictures from a negative design, which comprises exposing to light under the design a light-sensitive material sensitized by means of a mixture of silver nitrate and 4-diazodiphenylamine, subjecting the picture thus obtained to the action of a substance of alkaline action and then to a fixing process.

8. A process of preparing positive pictures from a negative design, which comprises exposing to light under the design a light-sensitive material sensitized by means of a mixture of silver nitrate and 1-diazo-4-aminobenzene, subjecting the picture thus obtained to the action of a substance of alkaline action and then to a fixing process.

9. Light-sensitive material sensitized by means of a water-soluble silver salt and a light-sensitive aromatic diazo compound, the light decomposition products of which have reducing properties for the exposed silver salt, the silver salt being used in sufficient quantity to produce a silver picture.

10. Light-sensitive material sensitized by means of a water-soluble silver salt and a light-sensitive aromatic diazo compound, which is substituted in the para-position to the diazo group by an amino group, the silver salt being used in sufficient quantity to produce a silver picture.

11. A process of preparing positive pictures from a negative design, which comprises exposing

15

20

25

30

35

40

45

50

55

60

65

70

75

to light under the design a light-sensitive material sensitized by means of a mixture of a water-soluble silver salt and a light-sensitive aromatic diazo compound, the light decomposition products 5 of which have reducing properties for the exposed silver salt, the silver salt being used in sufficient quantity to produce a silver picture, and subjecting the picture thus obtained to the action of a substance of alkaline action and then to a fixing 10 process.

12. A process of preparing positive pictures from a negative design, which comprises exposing to light under the design a light-sensitive material sensitized by means of a water-soluble silver 15 salt and a light-sensitive aromatic diazo compound, which is substituted in the para-position to the diazo group by an amino group, the silver salt being used in sufficient quantity to produce a silver picture, and subjecting the picture thus 20 obtained to the action of a substance of alkaline action and then to a fixing process.

13. Light-sensitive material sensitized by means of a water-soluble silver salt and a light-sensitive diazo compound of the benzene series conforming 25 to the following structural formula:



30 wherein X stands for a diazo group, Y stands for a member of the group consisting of hydrogen

and an alkyl-amino group, and Z stands for a member of the group consisting of hydrogen, hydroxy, amino, alkyl-amino, and aryl-amino of the benzene series, only one of the substituents Z and Y standing for hydrogen, the silver salt being used in sufficient quantity to produce a silver picture. 5

14. A process of preparing positive pictures from a negative design, which comprises exposing to light under the design, a light-sensitive material 10 sensitized by means of a water-soluble silver salt and a light-sensitive diazo compound of the benzene series conforming to the following structural formula:



wherein X stands for a diazo group, Y stands for a member of the group consisting of hydrogen and an alkyl-amino group, and Z stands for a member of the group consisting of hydrogen, hydroxy, amino, alkyl-amino, and aryl-amino of the benzene series, only one of the substituents Z and Y standing for hydrogen, the silver salt being used 20 in sufficient quantity to produce a silver picture and subjecting the picture, thus obtained, to the action of a substance of alkaline action and, then, 25 to a fixing process.

GOTTLIEB VON POSER. 30  
ROBERT FRANKE.